

1

2,921,902

## LUBRICATING COMPOSITION CONTAINING A SYNERGISTIC EXTREME PRESSURE ADDITIVE

Harold J. Watson, Fishkill, N.Y., assignor to Texaco Inc., a corporation of Delaware

No Drawing. Application June 3, 1957  
Serial No. 662,992

6 Claims. (Cl. 252—33.6)

This invention relates to an improved lubricating composition containing a combination of additives which exhibits synergistic extreme pressure properties. More particularly, this invention relates to mineral oils containing a mixture of a chlorinated high molecular weight hydrocarbon and a metal dialkyl dithiocarbamate as an extreme pressure additive mixture.

The need for improved lubricating oils exhibiting extreme pressure properties increases continually as industrial machinery is subjected to increasingly heavier loads and as performance standards are raised higher. Recently, the need for lubricants possessing extreme pressure properties has arisen in connection with turbine oils employed in the lubrication of marine machinery. A recently issued military specification, MIL-L-17331A(Ships), defines the desired properties of an extreme pressure turbine oil. The present invention defines an additive combination possessing synergistic extreme pressure action which is particularly useful in the formulation of marine extreme pressure turbine oils.

The synergistic extreme pressure additive combination of this invention consists essentially of a chlorinated paraffin wax and a metal dialkyl dithiocarbamate in a weight ratio of 5 to 500 parts of chlorinated paraffin wax per part of metal dialkyl dithiocarbamate. The lubricating compositions of the invention comprise 0.5 to 5.0 weight percent chlorinated paraffin wax and 0.002 to 0.1 weight percent metal dialkyl dithiocarbamate. Very small concentrations of metal dialkyl dithiocarbamates, which have substantially no extreme pressure properties in themselves, cause a significant and substantial improvement in the extreme pressure properties of chlorinated paraffin wax.

With the addition of conventional anti-oxidant, anti-foam, and anti-rust additives, extreme pressure turbine lubricants meeting the rigid requirements of MIL-L-17331A(Ships) were formulated using the synergistic extreme pressure additive combination of this invention.

The mineral lubricating base oil employed in the lubricant compositions of this invention may be derived from paraffin base, napthene base or mixed paraffin-naphthene base crudes. The viscosity range of the mineral lubricating base oil is between 80 and 1000 SUS at 100° F. The base oils usually have a flash point falling between 320 and 520° F., a pour point within the range of +20 to -50° F. and a viscosity index between 10 and 120.

Particularly preferred oils for marine turbine lubricants are paraffin base distillate oils which have been solvent refined, solvent dewaxed and clay percolated and which have an SUS at 100° F. between 300 and 600. A blend of furfural refined, acid-treated, clay-contacted solvent dewaxed and clay percolated paraffin base distillate oils having an SUS at 100° F. of 500-510, a pour of -10° F., a flash above 350° F., and a viscosity index of about 90 has been widely used as a base oil for marine turbine oils.

The chlorinated paraffin wax employed in the present lubricant is one having a high content of combined chlorine, the major proportion of which is in a so-called

2

active state. The chlorine content of this additive is between 35 and 45 weight percent of the compound. For example, a preferred material of this character has a total combined chlorine content of about 40-45 percent with an active chlorine content of about 29-34 percent. Preferably, the chlorinated paraffin wax contains a small proportion of an oil-soluble corrosion inhibitor of the type disclosed in U.S. Patent No. 2,298,638, which functions to neutralize the effect of any decomposition of the chlorinated paraffin wax with the release of free chlorine. Phenoxyl propylene oxide is used as a corrosion inhibitor of this type.

The concentration of the chlorinated paraffin wax in the lubricant composition of the invention falls between 0.5 and 5.0 weight percent of the total lubricant with concentrations between 1.0 and 2.5 weight percent usually being employed. It is significant that the desired level of extreme pressure activity is obtained with relatively low concentrations of chlorinated paraffin wax, which fact is directly attributable to the synergistic action of the metal dialkyl dithiocarbamate.

The metal dithiocarbamates which are employed as the second component of the additive combination of our invention are zinc and cadmium salts of organic-substituted dithiocarbamic acids having the general formula



wherein R and R' are aliphatic hydrocarbon radicals containing 2 to 14 carbon atoms and M is zinc or cadmium. Zinc dialkyl dithiocarbamates are particularly useful. Examples of suitable compounds are zinc dibutyl dithiocarbamate, zinc diethyl dithiocarbamate, zinc di(2-ethylhexyl) dithiocarbamate, zinc octyl-butyl dithiocarbamate, cadmium propyl-octyl dithiocarbamate, zinc diethyl dithiocarbamate, zinc dinonyl dithiocarbamates, cadmium diethyl dithiocarbamate, cadmium dibutyl dithiocarbamate and cadmium diethyl dithiocarbamate.

Only small concentrations of zinc and cadmium dialkyl dithiocarbamates are necessary to exert their synergistic action on the extreme pressure properties of chlorinated paraffin wax. Concentrations as low as 0.002 to 0.1 weight percent metal dialkyl dithiocarbamate based on the total lubricating oil composition effect a substantial improvement in the extreme pressure properties of a lubricating oil containing 0.5 to 3.0 weight percent chlorinated paraffin wax. The concentration of the metal dialkyl dithiocarbamate in the finished commercial lubricants is usually between 0.008 and 0.05 weight percent.

The weight ratio of chlorinated paraffin wax to metal dialkyl dithiocarbamate in the synergistic extreme pressure additive of the invention expressed independently of the mineral lubricating oil is 5 to 500 and preferably 50 to 300 parts of chlorinated paraffin wax per part of metal dialkyl dithiocarbamate. This ratio indicates very clearly the effectiveness of metal dialkyl dithiocarbamates in synergistically raising the extreme pressure property of chlorinated paraffin wax.

Alkyl-substituted phenols are usually incorporated in the lubricants of the invention as anti-oxidants. The preferred and most commonly used alkyl phenol anti-oxidant is 2,6-di-tertiary butyl-4-methylphenol which is commercially available from a number of sources. Examples of other phenolic type anti-oxidants which may be employed are 2,6-di-tertiary butylphenol; 2,6-di-tertiary amyl-4-methylphenol; and 2,6-di-isopropyl-4-methylphenol. Hindered phenols of this type are employed in concentrations between 0.1 and 1.0 weight percent.

Although hindered phenol type anti-oxidants are the most widely used anti-oxidants in the lubricant composi-

tions of the invention, aryl-substituted amine anti-oxidants such as phenylalphanaphthylamine, paraphenylenediamine, and diphenylamine are also used in lubricants in conjunction with the synergistic extreme pressure additive combination of the invention. The amine anti-oxidants are employed in the same concentrations as the hindered phenol anti-oxidant.

The anti-rust compounds which are particularly necessary for marine turbine lubricants are the alkyl-substituted aliphatic dicarboxylic acids such as alkenyl succinic acid, alkyl maleic acid and alkyl succinic acids. These aliphatic-substituted dicarboxylic acids are usually used in conjunction with a minor portion of an acid ester of an alkyl phosphate. A mixture of mono- and dilauryl esters of phosphoric acid is widely used in conjunction with an aliphatic-substituted aliphatic dicarboxylic acid as an anti-rust additive mixture. A detailed description of this additive mixture is found in U.S. Patent 2,452,321, which issued October 26, 1948, to J. A. Patterson and H. D. Kluge, and which is assigned to The Texas Company. The dicarboxylic acid is usually employed in a concentration between 0.01 and 0.1 weight percent and the alkyl acid phosphate in a concentration between 0.0001 and 0.03 weight percent.

Organic silicones are normally incorporated in the lubricants of the invention to impart anti-foam properties thereto. The silicones are usually of dialkyl or mixed alkyl-aryl silicone type. Dimethyl silicone is normally employed as the anti-foam agent. The silicone is incorporated in the lubricant by means of a kerosene concentrate containing 5 to 15 weight percent silicone. A very satisfactory anti-foam agent is kerosene concentrate containing 10 weight percent dimethyl silicone. The kerosene concentrate is employed in an amount of 0.005 to 0.025 weight percent which is sufficient to provide a silicone polymer concentration of 50 to 200 parts per million.

The synergistic extreme pressure properties of an additive mixture of chlorinated paraffin wax and zinc dialkyl dithiocarbamate was demonstrated in a base oil comprising mineral lubricating oil; 0.3 weight percent, 2,6-di-t-butyl-4-methylphenol; 0.033 weight percent of an anti-rust concentrate comprising 45 percent of a  $C_{12}$  alkenyl succinic acid in which the alkenyl group is propylene tetramer, 10 percent of a mixture of mono- and dilauryl phosphoric acid esters and 45 percent diluent oil; and about 0.001 weight percent of an anti-foam concentrate comprising 10 weight percent dimethyl silicone in kerosene. The mineral lubricating oil was a furfural refined, acid-treated, clay-contacted, solvent dewaxed and clay percolated paraffin base distillate having an SUS viscosity at 100° F. of about 500, a pour of -10° F. maximum, a flash of 380° F. minimum and a viscosity index of about 90.

In Table I, there are presented data proving the synergistic extreme pressure action of a mixture of zinc dialkyl dithiocarbamate and chlorinated paraffin wax having a chlorine content of 40 weight percent.

Table I

| Concentration of Additive in Base Oil |                              |                                 | Mean Hertz Load, kg. |
|---------------------------------------|------------------------------|---------------------------------|----------------------|
| Chlorinated Paraffin Wax              | Zinc Dibutyl Dithiocarbamate | Cadmium Dibutyl Dithiocarbamate |                      |
| None                                  | None                         | None                            | 17                   |
| None                                  | 0.01                         | None                            | 17                   |
| None                                  | 0.05                         | None                            | 18                   |
| None                                  | 0.1                          | None                            | 20                   |
| 2.0                                   | None                         | None                            | 26                   |
| 3.0                                   | None                         | None                            | 31                   |
| 2.0                                   | 0.01                         | None                            | 31                   |
| 2.0                                   | 0.05                         | None                            | 35                   |
| None                                  | None                         | 1.0                             | 22                   |
| 2.0                                   | None                         | 0.01                            | 28                   |

The data in the foregoing table prove that mixtures of chlorinated paraffin wax and zinc or cadmium dibutyl dithiocarbamate possess a surprising synergistic extreme pressure action. Although zinc butyl dithiocarbamate in a concentration of 0.01 percent had no effect on the mean Hertz load of the base oil and chlorinated paraffin wax in a concentration of 2.0 weight percent raised the mean Hertz load from 17 to 26, an additive combination of 0.01 weight percent zinc dibutyl dithiocarbamate and 2.0 weight percent chlorinated paraffin wax gave a mean Hertz load of 31. It is also significant that a mixture of 2.0 weight percent zinc dibutyl dithiocarbamate gave a mean 2.0 weight percent chlorinated paraffin wax and 0.01 Hertz load equivalent to that obtainable with 3.0 weight percent chlorinated paraffin wax and that a mixture of 2.0 weight percent chlorinated paraffin wax and 0.05 weight percent zinc dibutyl dithiocarbamate gave a mean Hertz load of 35, which is significantly higher than the 31 value obtained with 3.0 weight percent chlorinated paraffin wax alone.

Employing the synergistic extreme pressure additive combination of this invention, there has been formulated a finished lubricant which qualifies against MIL-L-17331A(Ships) for marine turbine lubricants containing extreme pressure properties; the composition of this product is shown in Table II.

Table II

|    | Lubricant composition<br>in weight percent                      |
|----|-----------------------------------------------------------------|
| 30 | Base oil 97.656                                                 |
|    | 2,6-di-t-butyl-4-methylphenol 0.3                               |
|    | C <sub>12</sub> alkenyl (propylene tetramer) succinic acid 0.03 |
|    | Mixture of mono- and dilauryl acid phosphates 0.003             |
| 35 | Chlorinated paraffin wax 2.0                                    |
|    | Zinc dibutyl dithiocarbamate 0.01                               |
|    | Anti-foam concentrate 0.001                                     |

40 The base oil in the above formulation is the same as that employed as the base oil for the data summarized in Table I. The chlorinated paraffin wax had a chlorine content of 40 weight percent.

45 In Table III, there are shown the properties of this lubricant in comparison with the specifications of MIL-L-17331A.

Table III

| Tests                                 | MIL-L-17331A        | Lubricant of Table II |
|---------------------------------------|---------------------|-----------------------|
| Flash, COC, ° F.....                  | 350 min.....        | 485                   |
| Viscosity:                            |                     |                       |
| cs. at 100° F.....                    | 82-110.....         | 109.3                 |
| SUS at 100° F.....                    | 506.6.....          | 506.6                 |
| cs. at 210° F.....                    | 8.2 min.....        | 10.8                  |
| SUS at 210° F.....                    | 62.2.....           | 62.2                  |
| Pour, ° F.....                        | 20 max.....         | 0                     |
| Corr. C.S. 212° F. (ASTM).....        | 1B max.....         | 1A                    |
| Neutrality, Qual.....                 | Must Pass.....      | Pass                  |
| Neut. No. (ASTM).....                 | 0.20.....           | 0.06                  |
| Emulsion, 130° F.:                    |                     |                       |
| Minutes.....                          | 30 max.....         | 30, 30                |
| cc. cufl.....                         | 3.....              | 2, 0                  |
| ASTM Foam, Seq. 1-2-3.....            | 300-25-300 max..... | 0-0-0                 |
| Ryder Gear Test, lb./in.....          | 2,200 min.....      | 1, 2, 790             |
| Mean Hertz Load, kg.....              | 25 min.....         | 31                    |
| Salt Water Rust Test (with wash)..... | Must Pass.....      | Pass                  |
| ASTM Oxidation, hrs. to 2 NN.....     | 1, 000 min.....     | 1, 2, 000             |

### 1. A *minimum of three*

Lubricant whose composition is shown in Table II has been evaluated as the turbine lubricant on the tanker "Indiana" for two months with excellent results.

70 "Indiana" for two months with excellent results.  
Obviously, many modifications and variations of the  
invention, as hereinbefore set forth, may be made without  
departing from the spirit and scope thereof and,  
therefore, only such limitations should be imposed as  
75 are indicated in the appended claims.

I claim:

1. A lubricating composition comprising a mineral lubricating oil as the major component, 0.5 to 5.0 weight percent chlorinated paraffin wax and 0.002 to 0.1 weight percent metal dialkyl dithiocarbamate in which said metal is selected from the group consisting of zinc and cadmium and said alkyl group contains 2 to 14 carbon atoms.

2. The lubricating composition of claim 1 containing 1.0 to 2.5 weight percent chlorinated paraffin wax and 0.008 to 0.05 weight percent metal dialkyl dithiocarbamate.

3. The lubricating composition of claim 1 in which said metal dialkyl dithiocarbamate is zinc dialkyl dithiocarbamate.

4. The lubricating composition of claim 1 in which said metal dialkyl dithiocarbamate is zinc dibutyl dithiocarbamate.

5. The lubricating composition of claim 1 in which said metal dialkyl dithiocarbamate is cadmium dibutyl dithiocarbamate.

6. A lubricating composition comprising a highly refined paraffin base distillate oil having an SUS at 100° F. between 300 and 600 as the major component, 0.5 to 5.0 weight percent chlorinated paraffin wax, 0.002 to 1.0 weight percent metal dialkyl dithiocarbamate in which the metal is selected from the group consisting of zinc and cadmium and said alkyl group contains 2 to 14 carbon atoms, 0.1 to 1.0 weight percent hindered phenol anti-oxidant, 0.01 to 1.0 weight percent alkenyl succinic acid, 0.0001 to 0.03 weight percent alkyl acid phosphate and 50 to 200 p.p.m. of a silicone polymer.

References Cited in the file of this patent

UNITED STATES PATENTS

|    |           |                      |               |
|----|-----------|----------------------|---------------|
| 15 | 2,394,536 | Denison et al. ----- | Feb. 12, 1946 |
|    | 2,400,106 | Denison et al. ----- | May 14, 1946  |
|    | 2,629,694 | Woods et al. -----   | Feb. 24, 1953 |
|    | 2,713,558 | Schmitz -----        | July 19, 1955 |
|    | 2,726,209 | Fainman -----        | Dec. 6, 1955  |